

# UNITED STATES PATENT OFFICE.

CLARK ALVORD, OF BINGHAMTON, NEW YORK.

## IMPROVEMENT IN BLACKINGS FOR BOOTS, &c.

Specification forming part of Letters Patent No. 160,741, dated March 16, 1875; application filed January 25, 1875.

*To all whom it may concern:*

Be it known that I, CLARK ALVORD, of the city of Binghamton, in the county of Broome and State of New York, have invented certain new and useful Improvements in Blacking for Boots, Shoes, Harness, and other Manufactures of Leather, of which the following is a specification:

My invention consists in compounding paraffine, bees-wax, and bone-black or lamp-black, or other suitable pigments, as follows, to wit: To one pound of hard paraffine add one-fourth pound of bees-wax; melt and stir them together, to which add one-fourth pound of bone-black or lamp-black, or enough to form a paste when thoroughly mixed by stirring and grinding with the liquid compound of paraffine and wax. When well mixed, let the compound cool, in the meantime forming it into rolls or balls of convenient size for use.

It is applied to use as follows: If the leather

is cold, slightly warm it; then rub the roll or ball over the same until slightly smeared; then polish by friction, using a brush or other suitable implement.

The proportions of materials above mentioned may be varied without producing injury. Therefore I do not intend to confine myself to the exact proportions above mentioned.

Having described my invention, I claim as new and desire to secure by Letters Patent—

The composition for blacking herein described, compounded of the materials substantially as above set forth.

In testimony that I claim the foregoing as my invention I hereunto affix my signature this 18th day of January, 1875.

CLARK ALVORD.

Witnesses:

CHAS. E. LEE,

LEWIS C. ALDRICH.